

## UNITED STATES PATENT OFFICE.

EUGEN VADERS, OF HEDDERNHEIM, NEAR FRANKFORT-ON-THE-MAIN, GERMANY.

## COPPER-ALUMINUM ALLOY.

No Drawing. Application filed March 31, 1927, Serial No. 180,064, and in Germany April 15, 1926.

This invention relates to copper-aluminum-alloys.

The heat resistance viz, strength in a heated state, of copper-aluminum alloys can be increased by additions of metals such as nickel, iron, manganese and the like. The addition of manganese imparts to these alloys the capability of being hot-pressed. If however the content of nickel and iron exceeds a certain limit, the alloy loses its capability of being pressed and is unable to regain same even if the manganese content is increased.

It has now been found possible to obtain copper-aluminum alloys which are capable of being pressed in a heated state by incorporating with said alloys, additions of 1 to 6% of manganese and 0.1 to 2% of tin, and if desired also small amounts of iron and nickel.

The amounts of the added iron and nickel should be so selected that the strength of the resulting alloy, in a heated state, is considerably increased while however the capability of the alloy of being pressed is not adversely affected.

By way of example alloys according to the present invention may consist of 5 to 9.5% aluminum, 1 to 6% manganese, 0 to 3% nickel, 0.1 to 3% iron and 0.01 to 2% tin, the remainder being copper.

The strength of an alloy consisting of 84 parts of copper, 9 parts of aluminum, 1 part of manganese, 3 parts of nickel and 3 parts of iron, at 500° C., is 35.7 kg. per sq. mm. If a small amount, e. g. 0.3 parts tin is added to this alloy the strength at the aforesaid temperature is increased to about 40 kg. per sq. mm.

Parallel with the increase in strength in

the heated state, an extraordinary increase 40 in the strength of the alloy at ordinary temperature takes place. An alloy consisting of 84 parts of copper, 9 parts of aluminum, 5 parts of manganese and 1.5 parts of iron was found to have a strength of 70.3 kg. 45 per sq. mm. at room temperature, and an elongation of 19.3%. If 0.5 parts of tin are added to the same alloy, the strength increases to more than 80 kg. per sq. mm., whereas the elongation is only reduced by 50 2.6%, the same still amounting to 16.7%. The samples were cast in chill moulds. The same alloy without the addition of tin, was found to have a strength of 35 kg. per sq. mm. at 500° C. and with an addition of 0.5 parts 55 of tin, a strength of more than 40 kg. per sq. mm.

The above described alloys may be used for any suitable purposes and have proved particularly useful as bearing metal. 60

What I claim is:

1. Copper - aluminum - alloys containing 5-9.5% aluminum manganese within the limits of 1 to 6% and tin within the limits of 0.01 to 2%. 65

2. Copper - aluminum - alloys containing small amounts of nickel and iron, 5 to 9.5% aluminum, 1 to 6% manganese and .01 to 2% tin.

3. An alloy consisting of 5 to 9.5% aluminum, 1 to 6% manganese, a small amount not exceeding 3% nickel, 0.1 to 3% iron and 0.01 to 2% tin, the remainder being copper. 70

4. An alloy, consisting of 84% copper, 1.5% iron, 5% manganese, 9% aluminum, 0.5% tin. 75

In testimony whereof I affix my signature.  
DR. EUGEN VADERS.